

1

2,923,595

## METHOD OF SOAKING ANIMAL HIDES AND SKINS

Rudi Heyden and Jürgen Plapper, Dusseldorf, Germany, assignors to Böhme Fettchemie G.m.b.H., Dusseldorf, Germany, a corporation of Germany

No Drawing. Application January 20, 1958  
Serial No. 709,768

Claims priority, application Germany January 22, 1957

4 Claims. (Cl. 8—94.18)

This invention relates to a novel method of soaking animal hides and skins involving the use of low-molecular mercapto-alkane-sulfonic acids or their salts in the soaking liquor.

It is well known that the soaking action of the soaking liquor upon animal hides and skins in the manufacture of leather articles can be substantially improved by modifying the soaking liquor with various additives. For example, the prior art describes soaking liquors which contain small quantities of sodium hydroxide, sodium sulfide, sodium sulfhydrate or sodium sulfite. However, because of their alkalinity, these additives produce undesirable swelling effects in the animal hide and permit the soaking action to proceed in a pH range in which the bacteria growth is substantially accelerated.

It is also well known that soaking can be accelerated by adding mercapto-carboxylic acids or their salts to the soaking liquor. However, the use of mercapto-carboxylic acid additives also has certain disadvantages in that the fiber agglutination in high-temperature-dried hides and skins cannot be sufficiently loosened within a reasonable period of time with the aid of such modified soaking liquors. The finished leather therefore has inadequate fullness, a hard feel and a coarse grain.

It is an object of the present invention to provide an improved method of soaking hides and skins which will make it possible to accomplish a sufficient loosening of the fiber agglutination within a relatively short period of time without undue swelling and within a pH range in which the bacteria growth is held at a minimum.

Other objects and advantages of the present invention will become apparent as the description thereof proceeds.

We have discovered that all of the above objects and improvements are achieved and that the shortcomings of the prior art are overcome by soaking hides and skins, and particularly those which are thick and difficult to soak through completely, in soaking liquors modified with mercapto-alkane-sulfonic acids or their water-soluble salts.

Examples of mercapto-alkane-sulfonic acids which are eminently suitable for this purpose are 2-mercaptopropane-sulfonic acid-1, 3-mercaptopropane-sulfonic acid-1, 3-mercaptopropane-sulfonic acid-1 and 4-mercaptopropane-sulfonic acid-1. The mercapto-alkane-sulfonic acids are preferably employed in the form of their water-soluble salts, such as their alkali metal or ammonium salts, or their salts formed with organic bases such as dimethylamine, triethanolamine and diethanolamine.

The soaking action of the modified soaking liquor upon the hides and skins may be further enhanced by adding anionic or non-ionic wetting agents thereto.

Optimum results are obtained where the mercapto-alkane-sulfonic acids or their salts are added to the soaking liquor in an amount ranging from 0.05 to 1.00 gm./liter. The wetting agents are preferably added in amounts ranging from 0.5 to 1.0 gm./liter.

In addition to the advantages previously mentioned,

2

the mercapto-alkane-sulfonic acids have the advantage over the mercapto-carboxylic acids that the former are effective at considerably lower concentrations. Despite such low effective concentrations the soaking rate of the soaking liquors modified with the mercapto-alkane-sulfonic acids or their water-soluble salts according to the present invention is substantially greater than that of soaking liquors modified with mercapto-carboxylic acids or their salts.

10 The following examples will further illustrate the present invention and enable others skilled in the art to understand the invention more completely. It should be understood, however, that we do not wish to limit our invention to the particular examples given herein.

### Example I

Dried goat skins were drum-soaked in an aqueous solution containing 0.1 gm./liter of the triethanolamine salt of 4-mercaptopropane-sulfonic acid-1. After about three days the skins were thoroughly soaked through, as evidenced by a water absorption of about 124% by weight based on the weight of the dry skins.

As comparison, dried goat skins were soaked for three days in an aqueous solution containing 0.5 gm./liter sodium thioglycolate. The water absorption was only 107% by weight based on the weight of the dry skins.

### Example II

Sun-dried buffalo skins were soaked in an aqueous solution containing 0.5 gm./liter of the dimethylamine salt of 3-mercaptopropane-sulfonic acid-1 and 0.2 gm./liter of a commercial alkylsulfonate wetting agent. After about two days of soaking, the raw hides were thoroughly and uniformly soaked through and the fiber agglutination was excellently loosened.

The same results were obtained when 0.2 gm./liter of a commercial alkylbenzene sulfonate was added as a wetting agent instead of the alkylsulfonate.

### Example III

0.2 gm./liter of the sodium salt of 2-mercaptopropane-sulfonic acid-1 are used instead of the triethanolamine salt of 4-mercaptopropane-sulfonic acid-1 of Example I with an analogous soaking effect.

### Example IV

0.5 gm./liter of the ammonium salt of 4-mercaptopropane-sulfonic acid-2 are used instead of the mercapto-alkane-sulfonic acid salt of Example I with a good soaking action.

### Example V

0.1 gm./liter of the diethanolamine salt of 4-mercaptopropane-sulfonic acid-2 are used instead of the mercapto-alkane-sulfonic acid salt of Example II with a remarkable soaking effect.

### Example VI

0.75 gm./liter of the potassium salt of 4-mercaptopropane-sulfonic acid-2 are used instead of the mercapto-alkane-sulfonic acid salt of Example II with a good soaking effect.

While we have illustrated the present invention with the aid of certain specific embodiments, it will be readily apparent to those skilled in the art that the invention is not limited to these embodiments, and that various changes and modifications may be made without departing from the spirit of the invention or the scope of the appended claims.

70 We claim:

1. The method of soaking raw animal hides and skins, which comprises immersing said hides and skins in an

aqueous solution having dissolved therein from 0.05 to 1.00 gm./liter of compounds selected from the group consisting of mercapto-lower alkane-sulfonic acids and their water-soluble salts.

2. The method of soaking raw animal skins and hides, which comprises immersing said skins and hides in an aqueous solution having dissolved therein from 0.05 to 1.00 gm./liter of a compound selected from the group consisting of mercapto-lower alkane-sulfonic acids and their water-soluble salts, and from 0.5 to 1.0 gm./liter of 10 wetting agent selected from the group consisting of anionic and non-ionic wetting agents.

3. The method of soaking dried goat skins, which comprises immersing said goat skins in an aqueous solution having dissolved therein 0.1 gm./liter of the triethanol-15 amine salt of 4-mercapto-butane-sulfonic acid-1.

4. The method of soaking dried buffalo hides which comprises immersing said hides in an aqueous solution having dissolved therein 0.5 gm./liter of the dimethyl-amine salt of 3-mercapto-propane-sulfonic acid-1 and 0.2 gm./liter of a sulfonate wetting agent selected from the group consisting of alkylsulfonates and alkylbenzene sulfonates.

References Cited in the file of this patent

UNITED STATES PATENTS

2,615,828 Haefele ----- Oct. 28, 1952

OTHER REFERENCES

Progress in Leather Science, 1920-1945, Br. Manuf., Leather Asso., London, 1948, pp. 138 and 139.